

# UNITED STATES PATENT OFFICE.

CLEMENT L. PERKINS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,240,599.

Specification of Letters Patent. Patented Sept. 18, 1917.

No Drawing.

Application filed August 2, 1917. Serial No. 184,055.

To all whom it may concern:

Be it known that I, CLEMENT L. PERKINS, a citizen of the United States, residing at Pittsburgh, in the county of Allegheny, State of Pennsylvania, have invented certain new and useful Improvements in Flotation of Minerals, and I do hereby declare the following to be a full, clear, and exact description of the invention, such as will enable others skilled in the art to which it appertains to make and use the same.

This invention relates to the concentration of minerals, such as sulfid ores and the like, (for example, chalco-pyrite with a silicious gangue), by flotation, and is based upon the discovery that improved results can be obtained by carrying out the flotation operation with the addition to the ore or mineral pulp of alpha- or beta-naphthol, or a mixture thereof, either alone or with the addition of other agents promoting the flotation. The naphthols are non-oleaginous solid materials which can nevertheless be distributed throughout the ore pulp with such uniformity that minimum amounts are required for effecting the concentration of the mineral by flotation. It is not necessary that the chemically pure naphthols be used, but the commercial products can be used in their crude or unrefined state. These commercial products may consist largely or essentially of the individual alpha- or beta-naphthols, or of mixtures in varying proportions of the two naphthols.

In using the naphthols they may be added to the ore either alone or in admixture with other agents promoting the flotation, in any suitable manner, so that they will be thoroughly and uniformly distributed throughout the ore pulp. The mixture is then subjected to a flotation operation as in an ordinary Calow cell or in apparatus where the air is incorporated in the ore pulp by mechanical agitation.

The amount of the naphthol or naphthols used may vary somewhat, for example, between one-half pound or less and one and one-half pounds per ton of ore (that is, calculated on the weight of the ore and not of the ore pulp). It is characteristic of the invention that the froth obtained is readily broken up and the naphthols recovered therefrom so that they are available for use in the treatment of further amounts of ore. That is to say, the circuit water recovered

from the concentrate and even that recovered from the tailings contains notable amounts of the naphthol or naphthols which can be thus returned to the process with resulting economy in the amount required to be added for subsequent operations.

The naphthols may be used alone to promote the flotation operation and high grades of concentrates obtained; and the resulting concentrates can be much more easily separated by filtration than the common concentrates obtained by the use of oil as the flotation agent. The action of the naphthols may, however, be modified or supplemented by adding other agents (such as oils or non-oleaginous agents) which promote the flotation and which do not prejudicially affect the action of the naphthols.

In applying the naphthol or naphthols, they may be introduced into the tube mill in which the ore is being ground, or they may be otherwise introduced into the ore pulp in any suitable way, as, for instance, by first digesting in hot water and mixing the product with the ore pulp just before it enters the flotation cell.

I claim:

1. The method of effecting the concentration of minerals by flotation, which comprises adding to the mineral pulp a small amount of naphthol, and subjecting the resulting mixture to a flotation operation; substantially as described.

2. The method of effecting the concentration of minerals by flotation, which comprises adding to the mineral pulp a mixture of alpha- and beta-naphthols, and subjecting the resulting mixture to a flotation operation; substantially as described.

3. The method of effecting the concentration of minerals by flotation, which comprises adding to the mineral pulp a small amount of naphthol and other agents promoting the flotation, and subjecting the resulting mixture to a flotation operation; substantially as described.

4. The method of effecting the concentration of minerals by flotation, which comprises adding to the mineral pulp a small amount of naphthol and of oil, and subjecting the resulting mixture to a flotation operation; substantially as described.

In testimony whereof I affix my signature.

CLEMENT L. PERKINS.